

# UNITED STATES PATENT OFFICE.

THEODORE W. FRECH, JR., OF CLEVELAND, OHIO, ASSIGNOR TO GENERAL ELECTRIC COMPANY, A CORPORATION OF NEW YORK.

## TUNGSTEN MANUFACTURE.

1,089,757.

Specification of Letters Patent. Patented Mar. 10, 1914.

No Drawing.

Application filed October 9, 1912. Serial No. 724,825.

*To all whom it may concern:*

Be it known that I, THEODORE W. FRECH, Jr., a citizen of the United States, residing at Cleveland, in the county of Cuyahoga, State of Ohio, have invented certain new and useful Improvements in Tungsten Manufacture, of which the following is a specification.

My invention relates to the manufacture of tungsten for use in the filaments of incandescent electric lamps and for other purposes. Incandescent lamp filaments made of tungsten such as can be produced by my process can be operated on alternating current for an indefinite time without the transverse "faulting" or displacement of adjacent sections of filament known as "offsetting", and give very uniform and good results as regards length of life, maintenance of candle-power, and strength after burning. By this process, also, can be produced tungsten which possesses a greater or less degree of ductility and pliability even after prolonged exposure to high temperature, as in the incandescence of electric lamp filaments and of electric furnace resistors, etc. By my process, furthermore, can be produced coherent tungsten capable of mechanical working while hot and which if such hot working is sufficiently prolonged becomes freely capable of mechanical working and shaping when cold by reason of properties of ductility, malleability, pliability, etc., or, in general, of undergoing permanent deformation in any way under the application of force below the ultimate breaking strength of the material—acquired during the hot working or (if the material possessed any such properties before) greatly increased by a change in the material which occurs during the hot working. Different lots of such metal, also, exhibit great uniformity and reliability as regards their capacity for drawing down to the very finest sizes,—as for example, that required for a 10 watt 110 volt sign lamp. Tungsten produced in accordance with my invention and thus hot worked also tends when subjected to high temperature to retain the ductility, etc., acquired during the hot working,—or, at least, loses the same but gradually.

I have hereinafter described my process with particular reference to its employment for the production of coherent tungsten out of which electric lamp filaments are to be

made by swaging, rolling, drawing or other methods of mechanical working, as described in great detail in British Patents 23,499 of 1909 and 8031 of 1910 and in the patent to William D. Coolidge, No. 1,082,933, December 30, 1913, under the title of tungsten and methods of making the same for use as filaments of incandescent lamps and for other purposes, and assigned to the assignee of this application. As set forth in these British patents and in the U. S. patent above mentioned, the offsetting of tungsten filaments can be prevented by the addition of foreign material to the metal; and in particular, coherent tungsten possessing some or all of the properties above set forth has been produced from tungstic oxid ( $WO_3$ ) which has been fired in a Hessian or Battersea crucible, and also from powdered material to which have been added one or more of various refractory oxids such as those of thorium, zirconium, yttrium, erbium, didymium, or ytterbium, or substances which when decomposed by heating give such oxids, particularly thorium nitrate. The crucible firing, indeed, owes its efficacy in part to substances such as these (consisting largely of alumina and silica) found in the oxid after the firing and probably volatilized into it from the crucible, and in part to a coarsening of the tungstic oxid which results from the firing. While thoroughly efficacious and more reliable than the other modes of "addition" as heretofore employed, this firing treatment is expensive, because for the best results a crucible can be used only once and because when carried out at the most effective temperatures it generally involves the loss of a substantial amount of tungstic oxid by volatilization, and does not always produce a definite quantitative effect as to the amount of the "addition" thus made to the oxid.

My process possesses all the efficacy and reliability of the crucible firing above mentioned without any of its disadvantages, being simple, economical, easy to carry out and control, and perfectly definite in its effects. In this process, suitable substances or "addition" material whose introduction makes the metal filaments finally produced capable of incandescence on alternating current without offsetting (such as the oxids and compounds above referred to) are employed. This "addition" material is in

2  
troduced into the material from which the filaments are eventually to be produced at a suitable stage and the whole is then heated, especially good results being obtained when 5 this heating is carried out under oxidizing conditions. By this mode of procedure the effect of such substances in giving to the metal eventually obtained the property of not offsetting and of retaining its ductility even when highly heated is improved; and 10 the degree of coarseness or fineness of the tungsten—hitherto found to be a matter of considerable moment as regards the facility with which material to which such additions 15 as above mentioned have been made can be hot worked—ceases to be of prime importance. The treatment can advantageously be carried out with the compounds from which tungsten is produced, preparatory to 20 their reduction, though it can also be carried out in other ways. Superior results are obtained by employing thorium nitrate and introducing it into the material when the latter is in the form of tungstic oxid, and 25 afterward heating the oxid with this addition in an oxidizing atmosphere. This mode of procedure greatly intensifies and improves the final effects of the thorium nitrate addition as regards the non-offsetting properties 30 of the filament and its retention of ductility after high heating. The good results may possibly be due to some sort of chemical reaction between the tungstic oxid and the thorium nitrate, or to elimination of impurities present in the tungstic oxid; or it may 35 be that the thorium nitrate or the thorium under these conditions in some way facilitates some molecular or intermolecular change in the tungstic oxid; or the action 40 may be of some still different character, or a combination of various effects.

I will now describe in detail how my invention can be successfully carried out commercially. A satisfactory quality of tungstic oxid can be produced by dissolving tungstic oxid ( $WO_3$ ) as pure as commercially obtainable in ammonia water, purifying the ammonium tungstate thus formed by crystallization over a steam bath, and then, after 45 washing with distilled water and drying, decomposing the ammonium tungstate by the application of moderate heat, say 400° to 500° C., which drives off the ammonia and leaves tungstic oxid. Alternatively, 50 and with very good results, the ammonium tungstate solution may be precipitated with concentrated hydrochloric acid—care being taken in the addition of the hydrochloric acid to the solution not to pass the neutral 55 point—the resulting crystals of ammonium tungstate filtered off, washed with distilled water, and heated as before to convert to tungstic oxid.

The tungstic oxid purified as just described or in any adequate manner is mixed

with thorium nitrate solution. Though the proportions can be varied, good results are obtained by using, with a kilogram of tungstic oxid, 75 cubic centimeters of thorium nitrate solution of such strength that 10 70 cubic centimeters of it contain 1 gram of thorium oxid ( $ThO_2$ ). The weight of a thorium nitrate solution of this strength is 1.1484 times that of an equal volume of water, which fact affords a convenient test. 75 The mixture obtained by the addition of the thorium nitrate solution to the tungstic oxid as just described contains approximately three-fourths of one per cent. of thorium oxid by weight. To this mixture sufficient 80 water is added to make a thick solution or paste, which is thoroughly stirred over a water bath, so that the materials are thoroughly, intimately, and uniformly incorporated together. According to one mode of 85 procedure, this stirring over the water bath is continued until the material becomes a thick mud that can be molded like clay, and this mud is packed with a ram-rod into a tubular mold of about 1 $\frac{1}{8}$ " internal diameter 90 and about 10" long. The material is then pushed from the mold and the slug or rod thus obtained is dried in an ordinary gas oven until it will hold together sufficiently to bear handling. Alternatively, the heating 95 of the material over the water bath may be continued until it is evaporated to dryness and the tungstic oxid powder thus obtained may be pressed dry in a mold into a rectangular slug or briquet about 1" or 100  $\frac{3}{4}$ " square and 9" long, the mold being sufficiently reinforced to withstand high pressure and a hydraulic press being employed. It will be understood that the formation of the oxid into a slug in either of these ways 105 is merely to put it in a convenient form for the subsequent heating operation and to obviate the necessity of employing boats to contain the loose powder, since most of the materials which would be convenient for 110 such boats would be liable to contaminate it or would be rapidly deteriorated by it, or are unduly expensive.

The firing of the slug may conveniently be carried out in a porcelain tube furnace 115 about 24" long and of 1 $\frac{1}{2}$ " internal diameter electrically heated by a suitable external winding, the slug being pushed through this furnace at the rate of about 1" every four minutes. The ends of this furnace being open to the atmosphere, oxidizing conditions will exist within it without any special steps being taken to introduce oxidizing gas into it. The furnace may to advantage be maintained at such a temperature that its interior matches in color with the carbon filament of an ordinary carbon filament lamp operated at 45% of the voltage for which it would operate at the standard efficiency of 3.1 watts per candle. The 120 125 130

slugs shrink slightly during this firing operation, and when they come from the furnace they are green in color. This change in color may possibly be due to the formation of a low thorium tungstate or tungsten thoriate by reaction between the tungsten trioxid and the thorium nitrate, or to other causes.

The fired slug may be pulverized in an ore crusher and the oxid powder then reduced in a porcelain tube furnace electrically heated by an external platinum winding, hydrogen being passed over the surface of the oxid in the tube and the temperature 10 gradually raised until the interior of the furnace matches in color with the carbon filament of an ordinary carbon filament lamp burning at 45% of its voltage for a 15 3.1 watt per candle efficiency,—though a 20 temperature at which the interior of the tube will match with such a filament burning at 30% of the rated voltage as just stated will suffice. Alternatively, the slug 25 may be reduced with hydrogen in the same way without crushing; this will give a mass 30 of tungsten particles so soft and friable that it can be pulverized between the fingers. This mass may be reduced to powder in any suitable way, as by grinding in a porcelain mortar.

The tungsten powder obtained in any of the ways above indicated may be pressed up into a rod and worked into filament form or into any other desired shape as described in 35 the above mentioned British patents and the above patent of William D. Coolidge.

What I claim as new, and desire to secure by Letters Patent of the United States, is:—

1. The step in the manufacture of tungsten for use in incandescent lamp filaments which consists in adding to a tungsten bearing material a relatively small amount of a compound of thorium and heating the mixture under oxidizing conditions.

2. The process of preparing a compound 45 containing tungsten for subsequent reduction to tungsten and the drawing of the said tungsten down to wire which consists in heating said compound under oxidizing conditions with a compound of thorium. 50

3. The process of preparing an oxid of tungsten for subsequent reduction to tungsten and the drawing of the said tungsten down to wire which consists in heating said oxid under oxidizing conditions with a compound of thorium. 55

4. The process of preparing an oxid of tungsten for subsequent reduction to tungsten and the drawing of the said tungsten down to wire which consists in heating said oxid under oxidizing conditions with a compound of thorium which is broken up upon heating to produce an oxid of thorium. 60

5. The process of preparing tungstic oxid for subsequent reduction to tungsten and 65 the drawing of the said tungsten down to wire which consists in heating said oxid under oxidizing conditions with a compound of thorium.

6. The process of preparing tungstic oxid 70 for subsequent reduction to tungsten and the drawing of the said tungsten down to wire which consists in heating said oxid under oxidizing conditions with a compound of thorium which is broken up upon 75 heating to produce an oxid of thorium.

7. The method which consists in heating to a suitable temperature in an oxidizing atmosphere tungstic oxid with which is intimately incorporated a comparatively small 80 proportion of thorium nitrate.

In witness whereof, I have hereunto set my hand this 28th day of September, 1912.

THEODORE W. FRECH, JR.

Witnesses:

JOHN M. STRONG,  
RALPH B. HUNTER.